

## UNITED STATES PATENT OFFICE.

EMILE THEODORE JOSEPH WATREMEZ, OF BRUSSELS, BELGIUM.

## TREATMENT OF TEXTILE FIBERS FOR BLEACHING PURPOSES.

1,133,769.

Specification of Letters Patent.

Patented Mar. 30, 1915.

No Drawing.

Application filed February 6, 1914. Serial No. 817,060.

*To all whom it may concern:*

Be it known that I, EMILE THEODORE JOSEPH WATREMEZ, a citizen of the Republic of France, and resident of Brussels, Belgium, have invented a new and useful Treatment 5 of Textile Fibers for Bleaching Purposes, which is fully set forth in the following specification.

This invention relates to an improved 10 process for the preparation of textile fibers of vegetable origin, more particularly, but not exclusively, applicable to fibers difficult to bleach, of which flax is a typical example.

The improved process chiefly consists in 15 treating the natural coloring matters of the fiber with metal salts, the corresponding oxids of which are little, or not at all, soluble in water. Salts containing as the single metal an alkaline metal, are therefore excluded, apart from the cases where it is necessary to produce an alkaline medium. The treatment of the fiber eliminates to a great 20 extent the natural coloring matters, and renders easily destructible by the bleaching agents those which are not eliminated; it 25 comprises the following steps:

1. *Boiling.*—This operation must be carried out in an alkaline medium; the treatment is by a salt of a metal, the oxid of 30 which is soluble in an excess of alkali, such as zinc in the form of zinkate of soda, chromium in the form of chromate of potash, tin in the form of stannate of soda, and preferably aluminium in the form of aluminate of 35 soda; it is important that the excess of alkali should be always sufficient for insuring complete solution of the metal oxid.

The proportions vary of course with the 40 nature of the fibers to be treated, but nevertheless by way of example the following composition of a boiling bath of 1000 liters may be mentioned: 10 kg. of crystallized alum and 5 kg. of carbonate of soda are dissolved together, and when this operation is 45 completed, the precipitate, which is formed at such time, is dissolved in 20 liters of caustic soda lye at 32-36° Baumé, and the necessary water is added, the use of the carbonate of soda enabling a smaller quantity of caustic soda to be employed than would otherwise be essential. The fibers are then introduced and heated. Discoloration quickly begins long before the boiling temperature is reached. The boiling is continued for about 50 two hours, and the material treated is preferably left to cool in the bath used for boil-

ing. It is rinsed with running water, or with water slightly acidulated with hydrochloric acid for the purpose of eliminating the excess of alkali. 60

The operation is carried out in the same way as in ordinary boiling, but it is unnecessary to do the work in any autoclave boiler under pressure, as this latter treatment gives loss of weight which can be easily avoided. 65 The boiling is preferably done either in a "jigger" or in vats with stirring wheels. After this operation, a large portion of the coloring matter is eliminated, and the coloring matters still left, are in combination with the metal. If the oxid of the said metal is colorless, and if the fibers treated are easy to bleach, the bleaching operation can be at once proceeded with. 70

2. *Attack of metal salts existing in the fiber after the first operation.*—These metal salts are treated with one or more agents capable of destroying or modifying them. According to the metal or metals utilized for boiling, the treatment is effected with a 80 suitable acid, the concentration of the acid varying according as the operation is carried out hot or cold. As regards alumina good results are obtained by means of sulfuric acid at the rate of 2 or 3 per thousand. 85 The treatment could also be effected by means of other substances, such as alkaline sulfids; in such case it is advisable to destroy, by means of an acid, sulfur compounds which have been produced in the 90 fiber.

Generally speaking, this treatment is sufficient for obtaining perfect whiteness in a few hours at the outside when followed by passage through an ordinary chlorin bath of 95 medium or weak strength. Nevertheless, for certain fibers or certain fabrics specially difficult to bleach, a second treatment with a metallic salt solution is made use of; that is to say, before proceeding to bleaching, the 100 natural coloring matters remaining are again treated with a metal salt, after removal of the metal utilized in the first operation. For example, it is convenient to employ a solution of bisulfite of soda, of 0.6-1.2% mixed with 2-4 per thousand of hydrochloric acid containing in solution a metal such as copper, chromium or manganese. The whole is then rinsed with cold water, and passed through a chlorin bath 105 as before.

It must be pointed out that if the fiber is

treated with a copper or chromium salt, a beautiful bluish-white is obtained, the blue tints disappearing easily under the action of any substance such as nitric acid, capable of 5 dissolving the corresponding oxids. If manganese is used for treatment, the fiber remains colored yellow, the action of the chlorin bath is continued until the said tint is thoroughly uniform when viewed by transmitted light, and manganese oxid is removed, for instance, by means of sulfurous acid.

The process described has the advantage of being very economical, as the various manipulations are reduced to a minimum, the raw materials are very cheap and the treatment quick. A very pure white is obtained, and the loss in weight of the fabric is insignificant, for only the natural coloring materials of the fiber are attacked, and not their support, that is to say, cellulose, the latter being absolutely or almost absolutely intact.

Claims.

1. The herein-described process of treating textile fibers of vegetable origin previous to bleaching, which consists in subjecting the fibers to the action of an alkaline bath containing the salt of a metal, the oxid of which is soluble in the excess of alkali of 25 the bath, to attack the vegetable coloring matter and in destroying the metal salts remaining in the fibers.

2. The herein-described process of treating textile fibers of vegetable origin previous to bleaching, which consists in subjecting the fibers to the action of an alkaline bath containing the salt of a metal, the oxid 35

of which is soluble in the excess of alkali of the bath, to attack the vegetable coloring matter, and in treating the said fibers with 40 an acid of a concentration varying with the temperature of the bath to destroy the metal salts remaining therein.

3. The herein-described process of treating textile fibers of vegetable origin previous to bleaching, which consists in subjecting the fibers to the action of an alkaline bath containing the salt of a metal, the oxid 45 of which is soluble in the excess of alkali of the bath, to attack the vegetable coloring matter, and in successively treating the fibers with alkaline sulfids and with an acid of concentration varying in accordance with the temperature of the bath to destroy the metal salts remaining therein.

4. The herein-described process of treating textile fibers of vegetable origin previous to the bleaching, which consists in subjecting the fibers to the action of an alkaline bath containing the salt of a metal, the oxid 50 of which is soluble in the excess of alkali of the bath, to attack the vegetable coloring matter, and in destroying the metal salts remaining in the fibers, and in again subjecting the fibers to the action of the first-mentioned 55 bath containing the said metal salt, the oxid of which is soluble in an excess of alkali.

In testimony whereof I have signed this specification in the presence of two subscribing witnesses.

EMILE THEODORE JOSEPH WATREMEZ.

Witnesses:

CHARLES O. JOHNSON,  
EMILE VON WANSALS.